

Aug. 12, 1930.

W. S. MURRAY

1,772,840

## METHOD OF AND MEANS FOR ELECTROPLATING

Original Filed March 8, 1924 2 Sheets-Sheet 1



### Inventor

William S. Murray

By his Attorneys

Philip Sawyer Rice ~~et al.~~

Aug. 12, 1930.

W. S. MURRAY

1,772,840

METHOD OF AND MEANS FOR ELECTROPLATING

Original Filed March 8, 1924 2 Sheets-Sheet 2

Fig. 4.



Fig. 5.



Fig. 6.



Fig. 7.



Fig. 8.



Inventor

William S. Murray

By his Attorneys

Philip Dwyer, Richard Kennedy

## UNITED STATES PATENT OFFICE

WILLIAM S. MURRAY, OF UTICA, NEW YORK, ASSIGNOR TO ONEIDA COMMUNITY, LIMITED, OF ONEIDA, NEW YORK, A CORPORATION OF NEW YORK

## METHOD OF AND MEANS FOR ELECTROPLATING

Application filed March 8, 1924, Serial No. 697,708. Renewed July 28, 1927.

This invention relates to improvements in methods of and means for electro-depositing metals.

Heretofore the electro-deposition of metals upon the bases or objects to be plated has been accomplished by the use of a direct current of low voltage passing through the plating solution and maintained at a constant current density or amperage during the period of electro-deposition.

According to the present invention the current density is changed at regular, predetermined intervals, according to the object to be attained, which may be a desired color or density in the plating, greater speed in plating than is possible with the direct current of uniform density heretofore used, or the plating successively of a plurality of different metals.

20 The invention is of special importance for the plating of a plurality of metals and for this reason it will be described in detail in that connection although it is to be understood that it is not to be so limited.

25 The best potential for electrodepositing various metals varies according to the metal in question. The purpose of the present embodiment is to so vary the external resistance in the plating circuit that the best potential 30 and therefore the best current density for depositing these metals from the same solution may be obtained.

In the accompanying drawings—

Figure 1 is a plan view and Figure 2 a side elevation of a preferred form of mechanism embodying and for practicing the improvements of the present invention;

Figure 3 is a vertical section thereof on the line 3—3 of Figure 1, and Figures 4, 5, 6 and 7 are details of certain parts of said mechanism, which will be hereinafter fully described; and

Figure 8 is a diagrammatic view illustrating the way in which said mechanism is used for obtaining the results before referred to.

45 The mechanism shown includes a frame 1 having bearings 2 in which is journaled a shaft 3 which is driven, through a pulley 4 from any suitable source of power.

This shaft is provided with an enlargement 5 midway of its length and between said

enlargement and the ends of the shaft with two sets of discs 6—7 loosely mounted on the shaft so that they may be rotarily adjusted thereon and then locked in such adjusted position by means of nuts 8 which when screwed inwardly along the shaft force the discs towards the enlargement 5 which acts as an abutment for the discs and, with the nuts 8, securely locks them in their adjusted position.

In front of each of these two sets of discs 6—7 there is mounted a brush holder 9—9<sup>a</sup> and in said brush holder there is mounted a brush 10—10<sup>a</sup> which is pushed towards the discs by springs 11, its movement in its direction, however, being limited by stops 12. These two brushes 10 are connected by wires 13—14, respectively, and wire 15 with one terminal of a generator 16, the one terminal which is connected by a wire 17 with the cathode holder or terminal 18 of an electrolytic plating bath 19.

60 Wires 13—14 include resistances 20—21 of different values, the resistance 20 being weaker than the resistance 21.

65 On what may be termed the rear side of the machine, frame, there is mounted a second brush holder 22 and in this brush holder is mounted a brush 23 which is pressed outwardly by springs 24 into engagement with the enlargement 5 of shaft 3. This brush is connected by wire 25 with the anode holders or terminals 26 of the bath 19. These terminals are so arranged relatively to the cathode terminal 18, that the currents will flow from the anodes in different directions to the cathode.

70 The discs 6—7 have radially projecting portions 6<sup>a</sup>—7<sup>a</sup>, the surfaces of which are concentric with the axis of shaft 3.

75 The extent to which these said metal contacts project from shaft 3 is such that as said shaft rotates they will contact with brushes 10 and 10<sup>a</sup>, respectively, and thereby close the circuit from generator 16 through bath 19 by way of resistance 20 and brush 10, when the said metal contacts 6<sup>a</sup> of discs 6 are in engagement with said brush 10, or by way of resistance 21 and brush 10<sup>a</sup> when the segmental contacts 7<sup>a</sup> are in engagement with brush 10<sup>a</sup>.

80 It will be understood that the variation in 100

the relative strengths of these two resistances will result in corresponding changes in potentials and thereby densities of the currents through the bath 19. In the present case, the 5 resistance 20 is weaker than the resistance 21 with the result that the density or value of the current passing thence through the bath 19 will be greater when the current passes through 20 than the current passing through 10 resistance 21 to the bath.

15 The discs of each set 6—7 are, as before stated, relatively adjustable circumferentially on the shaft 3 so that their segmental contacts 6<sup>a</sup> or 7<sup>a</sup> may be aligned with each other axially on the shaft or be arranged spirally, or one in advance of another, around the shaft, as shown for example in the drawings. When so aligned, the duration of contact between segmental contacts 6<sup>a</sup> or 7<sup>a</sup>, as the case 20 may be, will continue for only a short time, namely for 7° 12" in the case of discs 6 and 36° in the case of discs 7.

25 When, however, these discs are adjusted with their segmental contacts spirally arranged around the shaft 3 the duration of contact may in the case of discs 6 be continued, without interruption, for 72°, and in the case of discs 7, for 360°.

It will thus be seen that with these two 30 sets of discs and the two brushes 10—10<sup>a</sup>, the current traversing the bath 19 may be pulsated to any desired degree, according to the character of the resistances, as 20—21, employed between the generator and the brushes 35 10—10<sup>a</sup>. This will depend upon the character of plating desired to be produced by the bath 19.

What is claimed is:

1. The combination with an electroplating 40 circuit including as a cathode the article to be plated, of means for periodically decreasing and increasing from one uniform value to another uniform value the density of the current passing through said cathode at regularly controlled intervals while maintaining the same sign of polarity of said current.

2. The combination with an electroplating circuit including as a cathode the article to be plated, of means for changing from one 50 uniform value to another uniform value the density of the current passing through said cathode at regularly controlled intervals while maintaining said current unidirectional.

3. The combination with an electroplating 55 circuit including as a cathode the article to be plated, of means for periodically and alternately flowing uni-directional electric currents of different uniform densities to the 60 cathode from anodes located in different directions from the cathode.

4. The combination with an electroplating circuit including as a cathode the article to be plated, of means for subjecting the plating 65 circuit to the action of a pulsatory, al-

ways uni-directional current which changes from one uniform value to another uniform value, and adjusting the duration and amplitude of the individual pulsations and the duration of the intervals between pulsations to give the desired coating on the article.

5. In a process of electroplating in which the article to be plated is included as a cathode in the plating circuit, the method of controlling the nature of the coating deposited on the article, which consists in periodically decreasing and increasing from one uniform value to another uniform value the density of the current passing through said cathode at regularly controlled intervals while maintaining said current always uni-directional.

6. In a process of electroplating in which the article to be plated is included as a cathode in the plating circuit, the method of controlling the nature of the coating deposited on the article, which consists in changing from one uniform value to another uniform value the density of the current passing through said cathode at regularly controlled intervals while maintaining said current always uni-directional.

7. In a process of electroplating in which the article to be plated is included as a cathode in the plating circuit, the method of controlling the nature of the coating deposited on the article, which comprises periodically and alternately flowing electric currents of different uniform densities to the cathode from anodes located in different directions from the cathode, said currents being uni-directional at all times and flowing in the same direction relative to the cathode.

8. In a process of electroplating in which the article to be plated is included as a cathode in the plating circuit, the method of controlling the nature of the coating deposited on the article, which comprises subjecting the plating circuit to the action of a pulsatory, always uni-directional current which changes from one uniform value to another uniform value, and adjusting the duration and amplitude of the individual pulsations and the duration of the intervals between pulsations to give the desired coating on the article.

In testimony whereof, I have hereunto set my hand.

WILLIAM S. MURRAY.

70

75

80

85

90

95

100

105

110

115

120

125

130